



US009605232B2

(12) **United States Patent**  
**Takagi et al.**

(10) **Patent No.:** **US 9,605,232 B2**  
(b4) **Date of Patent:** **Mar. 28, 2017**

(54) **WATER-SOLUBLE METALWORKING OIL AGENT, METALWORKING FLUID, AND METALWORKING METHOD**

(71) Applicant: **IDEMITSU KOSAN CO., LTD.**,  
Tokyo (JP)

(72) Inventors: **Fumiaki Takagi**, Chiba (JP); **Yoichiro Jido**, Chiba (JP)

(73) Assignee: **IDEMITSU KOSAN CO., LTD.**,  
Tokyo (JP)

(\*) Notice: Subject to any disclaimer, the term of this patent is extended or adjusted under 35 U.S.C. 154(b) by 257 days.

(21) Appl. No.: **14/359,194**

(22) PCT Filed: **Nov. 15, 2012**

(86) PCT No.: **PCT/JP2012/079661**

§ 371 (c)(1),  
(2) Date: **May 19, 2014**

(87) PCT Pub. No.: **WO2013/073615**

PCT Pub. Date: **May 23, 2013**

(65) **Prior Publication Data**

US 2014/0373584 A1 Dec. 25, 2014

(30) **Foreign Application Priority Data**

Nov. 17, 2011 (JP) ..... 2011-251924

(51) **Int. Cl.**

**C07C 55/02** (2006.01)  
**C10M 173/02** (2006.01)  
**C10M 169/06** (2006.01)  
**B21B 45/02** (2006.01)  
**C10M 169/04** (2006.01)  
**C10M 173/00** (2006.01)  
**C10M 101/00** (2006.01)  
**C10M 129/34** (2006.01)  
**C10M 129/44** (2006.01)  
**C10M 133/08** (2006.01)

(52) **U.S. Cl.**

CPC ..... **C10M 169/04** (2013.01); **C10M 173/00** (2013.01); **C10M 101/00** (2013.01); **C10M 129/34** (2013.01); **C10M 129/44** (2013.01); **C10M 133/08** (2013.01); **C10M 2203/106** (2013.01); **C10M 2203/1006** (2013.01); **C10M 2203/1065** (2013.01); **C10M 2207/123** (2013.01); **C10M 2207/125** (2013.01); **C10M 2207/126** (2013.01); **C10M 2207/128** (2013.01); **C10M 2207/281** (2013.01); **C10M 2207/283** (2013.01); **C10M 2207/285** (2013.01); **C10M 2207/2835** (2013.01); **C10M 2209/102** (2013.01); **C10M 2209/104** (2013.01); **C10M 2209/108** (2013.01); **C10M 2209/109** (2013.01); **C10M 2215/004** (2013.01); **C10M 2215/042** (2013.01); **C10M 2215/223** (2013.01); **C10N 2220/022** (2013.01); **C10N**

**2230/06** (2013.01); **C10N 2230/08** (2013.01); **C10N 2240/40** (2013.01); **C10N 2240/401** (2013.01); **C10N 2240/406** (2013.01); **C10N 2240/407** (2013.01); **C10N 2240/408** (2013.01); **C10N 2240/409** (2013.01); **C10N 2270/00** (2013.01)

(58) **Field of Classification Search**

CPC ..... C10N 2240/402; C10M 2207/123; C10M 2207/129; C10M 2207/125  
USPC ..... 508/506, 511, 519; 72/42  
See application file for complete search history.

(56) **References Cited**

U.S. PATENT DOCUMENTS

2012/0184475 A1 7/2012 Takagi et al.

FOREIGN PATENT DOCUMENTS

|    |              |         |
|----|--------------|---------|
| CN | 101970627 A  | 2/2011  |
| JP | 57 159891    | 10/1982 |
| JP | 60 141795    | 7/1985  |
| JP | 2-5799 B2    | 2/1990  |
| JP | 6-62981 B2   | 8/1994  |
| JP | 10 8077      | 1/1998  |
| JP | 10 195475    | 7/1998  |
| JP | 2000 63863   | 2/2000  |
| JP | 2000 256695  | 9/2000  |
| JP | 2002 146380  | 5/2002  |
| JP | 2011-79956 A | 4/2011  |
| JP | 2011 111593  | 6/2011  |
| WO | 2011 065355  | 6/2011  |

OTHER PUBLICATIONS

International Search Report Issued Feb. 19, 2013 in PCT/JP12/079661 Filed Nov. 15, 2012.

(Continued)

Primary Examiner — Vishal Vasisth

(74) Attorney, Agent, or Firm — Oblon, McClelland, Maier & Neustadt, L.L.P.

(57) **ABSTRACT**

The invention provides a water-soluble metal-working oil agent, including a component A and a component B, wherein the component A is a mineral oil which has a characteristic temperature, as measured in accordance with JIS K2242, of 570° C. or higher, and the component B is at least one condensed fatty acid which is selected from a condensed fatty acid (1), produced through dehydration condensation of a hydroxycarboxylic acid, and a condensed fatty acid (2), produced through dehydration condensation of an alcoholic hydroxyl group of the condensed fatty acid (1) with a monovalent carboxylic acid, which has a characteristic temperature, as measured in accordance with JIS K2242, of 650° C. or higher. The agent can provide excellent workability with a hard-to-work material and can prolong tool life.

(56)

**References Cited**

**OTHER PUBLICATIONS**

Combined Chinese Office Action issued Jun. 2, 2015 in Patent Application No. 201280056609.X (with English translation of categories of cited documents).

U.S. Appl. No. 14/359,209, filed May 19, 2014, Takagi, et al.

Kenjiro Hara, "Studies on the Change of Quenching Properties by the Temperature of Mineral Oil" Journal of Japan Society of Lubrication Engineers, vol. 8, No. 3, 1958, 5 Pages (with English Abstract).

**WATER-SOLUBLE METALWORKING OIL  
AGENT, METALWORKING FLUID, AND  
METALWORKING METHOD**

This application is a 371 of PCT/JP12/79661, filed Nov. 15, 2012.

TECHNICAL FIELD

The present invention relates to a water-soluble metal-working oil agent, for use in metal working; i.e., cutting or grinding of metal pieces, to a metal-working liquid, and to a metal-working method.

BACKGROUND ART

In metal machining processes such as cutting and grinding, a metal-working oil agent is used for improving machining efficiency, for preventing abrasion between a workpiece and a tool for machining the workpiece, for prolonging tool life, for removing metal chips, and for other purposes. Such metal metal-working oil agents include an oil-base agent predominantly containing an oil component such as mineral oil, animal and vegetable oil, or synthetic oil, and a water-soluble agent containing an oil component and a surface active compound. From the viewpoints of effective utilization of resources and fire prevention, a water-solubility-imparted agent (i.e., a water-soluble metal-working oil agent) has come to be used more and more in recent years.

In order to satisfy defoaming property and rotting resistance which are essential properties of the water-soluble metal-working oil agent and also to enhance machining efficiency, one proposed solution is incorporation of a compound, such as risinoleic acid polymer amine salt, into a metal-working oil agent (see Patent Document 1). Conventionally, chlorinated paraffin has been incorporated into a metal-working oil agent for the purpose of enhancing machining efficiency. However, since such a halohydrocarbon possibly generates dioxin, which is harmful to the human body, in recent years, a compound such as a sulfur compound or a phosphorus compound is used instead of chlorinated paraffin (see Patent Document 2). Furthermore, in order to attain further enhanced workability, there has been proposed incorporation, into a metal-working oil agent, of a compound such as a condensed risinoleic fatty acid, an ester compound, or an amine (see Patent Document 3).

However, as disclosed in Patent Documents 1 and 3, even in the case of a metal-working oil agent composed of a mixture of a risinoleic acid polycondensation product amine salt and a mineral oil, when a material which is difficult to work; i.e., hard-to-work material, such as titanium alloy, nickel alloy, or cobalt alloy, is subjected to cutting work, the heat generated during the working accumulates in a tool, and such an increased heat load causes problems, including shortening of tool life.

In another case where cutting speed is elevated to enhance productivity, higher heat is generated, and the heat imposes a further load on the tool. Thus, even in the case disclosed in Patent Document 3, where a risinoleic-acid-polycondensed fatty acid and an ester compound are used in combination, sufficient workability may fail to be attained. In the

case disclosed in Patent Document 2, use of a sulfur compound or a phosphorus compound may impose a load on the environment.

Therefore, in machining hard-to-work materials, there is demand for further improvement of a metal-working oil agent.

PRIOR ART DOCUMENTS

Patent Documents

Patent Document 1: Japanese Patent Application Laid-Open (kokai) No. Sho 57-159891  
Patent Document 2: Japanese Patent Application Laid-Open (kokai) No. Sho 60-141795  
Patent Document 3: Japanese Patent Application Laid-Open (kokai) No. 2011-111593

SUMMARY OF THE INVENTION

Problems to be Solved by the Invention

Thus, an object of the present invention is to provide a water-soluble metal-working oil agent, a metal-working liquid, and a metal-working method, which attain excellent workability with a hard-to-work material and which can prolong tool life.

Means for Solving the Problems

The present inventors have conducted extensive studies, and have found that the above object can be attained by selectively incorporating, into a water-soluble metal-working oil agent, as lubrication components, a mineral oil having a characteristic temperature meeting a specific condition, and a specific condensed fatty acid. The present invention has been accomplished on the basis of this finding.

Accordingly, the present invention is directed to the following:

[1] A water-soluble metal-working oil agent, characterized by comprising a component A and a component B, wherein:

the component A is a mineral oil which has a characteristic temperature, as measured in accordance with JIS K2242, of 570° C. or higher; and

the component B is at least one condensed fatty acid which is selected from a condensed fatty acid (1), produced through dehydration condensation of a hydroxycarboxylic acid, and a condensed fatty acid (2), produced through dehydration condensation of an alcoholic hydroxyl group of the condensed fatty acid (1) with a monovalent carboxylic acid, and which has a characteristic temperature, as measured in accordance with JIS K2242, of 650° C. or higher.

[2] A metal-working liquid comprising the water-soluble metal-working oil agent diluted by water.

[3] A metal-working method comprising working a metal workpiece by use of the water-soluble metal-working oil agent.

[4] A metal-working method comprising working a metal workpiece by use of the metal-working liquid.

Effects of the Invention

The present invention enables provision of a water-soluble metal-working oil agent, a metal-working liquid, and

a metal-working method, which attain excellent workability with a hard-to-work material and which can prolong tool life.

### MODES FOR CARRYING OUT THE INVENTION

The present invention will next be described in detail. [Water-Soluble Metal-Working Oil Agent]

An embodiment of the water-soluble metal-working oil agent includes a component A and a component B. The component A is a mineral oil which has a characteristic temperature, as measured in accordance with JIS K2242, of 570° C. or higher. The component B is at least one condensed fatty acid which is selected from a condensed fatty acid (1), produced through dehydration condensation of a hydroxycarboxylic acid, and a condensed fatty acid (2), produced through dehydration condensation of an alcoholic hydroxyl group of the condensed fatty acid (1) with a monovalent carboxylic acid, which has a characteristic temperature, as measured in accordance with JIS K2242, of 650° C. or higher.

The water-soluble metal-working oil agent may further contain a carboxylic acid as a component C. Also, the water-soluble metal-working oil agent may further contain an amine compound or an alkali metal compound, as a component D.

In the embodiment of the present invention, the term "water-soluble metal-working oil agent" refers to a cutting oil agent having water solubility that allows the agent to be diluted with water upon use of metal working. As used herein, the water-soluble metal-working oil agent refers to that in an undiluted state.

According to JIS K2242 (heat-treating oil quench test (method A)), the cooling process of a silver test probe is defined as a vapor step, a boiling step, and a convection step. The characteristic temperature refers to a temperature of transition from the vapor step to the boiling step.

More specifically, in the vapor step, the surface temperature of the heated test probe is high, and the test probe is covered with a vapor layer of the corresponding oil agent. That is, in the vapor step, the oil agent cannot come into direct contact with the test probe as a liquid. In other words, at a temperature equal to or higher than the characteristic temperature, the oil agent cannot act on the test probe as a liquid, and encounters difficulty in imparting lubricity to the test probe.

The boiling step corresponds to a state in which the oil agent comes into contact with the test probe after breakage of the vapor film, resulting in nuclear boiling. That is, in the boiling step, the oil agent can come into direct contact with the test probe as a liquid. In other words, at a temperature equal to or lower than the characteristic temperature, the oil agent can act on the test probe as a liquid, to thereby impart lubricity to the test probe.

#### <Component A>

The component A is a mineral oil having a characteristic temperature, as measured in accordance with JIS K2242, of 570° C. or higher. When the component A has a characteristic temperature lower than 570° C., an oil component involved in lubrication is readily vaporized, and a sufficient abrasion-reducing effect fails to be attained, resulting in shortened tool life. The characteristic temperature is preferably 590° C. or higher, more preferably 630° C. or higher. No particular limitation is imposed on the upper limit of the characteristic temperature, but it is preferably 800° C. or lower.

The aforementioned component A, which is a mineral oil having a characteristic temperature, as measured in accordance with JIS K2242, of 570° C. or higher, may be produced by, for example, removing a light fraction from a mineral oil through distillation under reduced pressure, to thereby adjust the kinematic viscosity at 40° C. of the component A to 300 mm<sup>2</sup>/s or higher, whereby the flash point of the component A is adjusted to 220° C. or higher. Thus, the component A having a characteristic temperature of 570° C. or higher can be obtained.

The kinematic viscosity of the component A, as measured at 40° C., is preferably 300 mm<sup>2</sup>/s or higher, more preferably 400 mm<sup>2</sup>/s or higher. When the component A has a kinematic viscosity as measured at 40° C. of 300 mm<sup>2</sup>/s, tool life can be effectively prolonged. No particular limitation is imposed on the upper limit of the kinematic viscosity of the component A, but is preferably 500 mm<sup>2</sup>/s or lower.

The flash point of the component A is preferably 220° C. or higher, more preferably 230° C. or higher. When the flash point is lower than 220° C., targeted characteristic temperature cannot be attained, and sufficient workability may fail to be attained.

Examples of the mineral oil which may be used in the present invention include distillates produced through distillation, under normal pressure, of paraffin base crude oil, middle crude oil, or naphthene base crude oil; distillates produced through distillation, under reduced pressure, of residual oil of normal-pressure distillation of paraffin base crude oil, middle crude oil, or naphthene base crude oil; and refined oils obtained by refining these distillates. Specific examples include solvent-refined oil, hydro-refined oil, dewaxed oil, and clay-treated oil.

Of these, a mineral oil originating from naphthene base crude oil is preferred, from the viewpoint of compatibility to a surfactant employed for imparting water solubility to the metal-working oil agent.

The component A is preferably contained in an amount of 10 mass % or more with respect to the entire amount of the water-soluble metal-working oil agent, more preferably in an amount of 15 mass % or more. When the component A content is 10 mass % or more, tool life can be sufficiently prolonged.

Notably, the kinematic viscosity of mineral oil is determined in accordance with JIS K2283; the density of mineral oil is determined in accordance with JIS K2249; and the flash point is determined in accordance with JIS K2265-4 (COC method).

#### <Component B>

The component B is at least one condensed fatty acid which is selected from a condensed fatty acid (1), produced through dehydration condensation of a hydroxycarboxylic acid, and a condensed fatty acid (2), produced through dehydration condensation of an alcoholic hydroxyl group of the condensed fatty acid (1) with a monovalent carboxylic acid, and has a characteristic temperature, as measured in accordance with JIS K2242, of 650° C. or higher.

When the characteristic temperature of the component B is lower than 650° C., the component B is readily vaporized, and a sufficient abrasion-reducing effect fails to be attained, resulting in shortened tool life. From these viewpoints, the characteristic temperature of the component B is preferably 670° C. or higher, more preferably 690° C. or higher.

An example of the hydroxycarboxylic acid for use in production of the component B having a characteristic temperature, as measured in accordance with JIS K2242, of 650° C. or higher is ricinoleic acid. The hydroxycarboxylic acid can be produced through dehydration polycondensation

## 5

of ricinoleic acid (12-hydroxyoctadeca-9-enonic acid). When ricinoleic acid heated to about 200° C. in an inert atmosphere, dehydration polycondensation initiates, to thereby yield a polycondensed fatty acid.

The ricinoleic acid polymerization degree is controlled by reaction time. The longer the reaction time, the lower the acid value and hydroxyl value. Thus, a fatty acid having a high polycondensation degree can be produced. The higher the polycondensation degree, the higher the characteristic temperature of the produced polycondensed fatty acid.

The condensed fatty acid (2) is produced by carrying out dehydration polycondensation of a dehydration polycondensation product of a hydroxycarboxylic acid with an additional monovalent carboxylic acid. Progress of this reaction can be confirmed by a drop in hydroxyl value. As a result of this reaction, a polycondensed fatty acid having a higher characteristic temperature can be produced.

The monovalent carboxylic acid used in the reaction may be a saturated or unsaturated carboxylic acid. However, a C $\geq$ 4 carboxylic acid is preferred, since a malodor and metal corrosion may be induced by an unreacted carboxylic acid having a few carbon atoms remaining in the reaction system. Examples of the saturated carboxylic acid include caproic acid, enanthic acid, caprylic acid, 2-ethylhexanoic acid, pelargonic acid, isononanoic acid, capric acid, neodecanoic acid, lauric acid, myristic acid, palmitic acid, stearic acid, arachidic acid, behenic acid, and lignoceric acid. Examples of the unsaturated carboxylic acid include undecylenic acid, oleic acid, elaidic acid, erucic acid, nervonic acid, linoleic acid,  $\gamma$ -linolenic acid, arachidonic acid,  $\alpha$ -linolenic acid, stearidonic acid, eicosapentaenoic acid, and docosahexanoic acid.

The component B preferably has an acid value of 60 mgKOH/g or less, more preferably 40 mgKOH/g or less. When the acid value of the component B is in excess of 60 mgKOH/g, a target characteristic temperature cannot be attained, and sufficient workability may fail to be attained.

The component B preferably has a hydroxyl value of 50 mgKOH/g or less, more preferably 35 mgKOH/g or less. When the hydroxyl value of the component B in excess of 50 mgKOH/g, a target characteristic temperature cannot be attained, and sufficient workability may fail to be attained.

The component B is preferably contained in an amount of 7.5 mass % or more with respect to the entire amount of the water-soluble metal-working oil agent, more preferably in an amount of 10 mass % or more. When the component B content is 7.5 mass % or more, a sufficient abrasion-reducing effect can be attained, thereby prolonging tool life.

Notably, the acid value is determined in accordance with JIS K2501; the hydroxyl value is determined in accordance with JIS K0070; and a saponification value is determined in accordance with JIS K2503.

## &lt;Component C&gt;

The water-soluble metal-working oil agent preferably contains a carboxylic acid serving as the component C. The carboxylic acid which may be used as the component C may be a unsaturated carboxylic acid or a saturated carboxylic acid and may have a linear-chain structure or a cyclic structure. The component C is preferably a C4 to C30 monovalent carboxylic acid, divalent carboxylic acid, or polyvalent carboxylic acid.

The same monovalent carboxylic acid as employed in production of the component B may be employed as the component C.

## 6

Examples of the divalent carboxylic acid include adipic acid, suberic acid, sebatic acid, azelaic acid, and dodecanoic acid. Examples of the polyvalent carboxylic acid include citric acid.

5 The carboxylic acid serving as the component C is contained in an amount of 2 mass % or more with respect to the entire amount of the water-soluble metal-working oil agent, preferably in an amount of 5 mass % or more, more preferably in an amount of 8 mass % or more. When the 10 component B content is less than 2 mass %, stability of the water-soluble metal-working oil agent and its diluted product may fail to be fully attained.

## &lt;Component D&gt;

15 The water-soluble metal-working oil agent preferably contains an amine compound or an alkali metal compound serving as the component D. From the viewpoint of stability of the water-soluble metal-working oil agent, the component D is preferably contained in such a neutralization equivalent that at least the component B and component C are neutralized to cancel out the sum of the acid values thereof. The upper limit of the component D content is such an amount that a 10 vol. % water-diluted product of the water-soluble metal-working oil agent has a pH of 11. When the component D content is less than the neutralization equivalent, the water-soluble metal-working oil agent has poor stability. When the diluted liquid has a pH in excess of 11, workers involved in metal working may suffer rough hands.

20 The amine compound which may be used as the component D may be a primary amine, a secondary amine, a tertiary amine, or an alkanolamine.

25 Examples of the primary amine include monoethanolamine, monopropanolamine, monoisopropanolamine, 2-amino-1-butanol, 2-amino-2-methylpropanol, butylamine, pentylamine, hexylamine, cyclohexylamine, octylamine, laurylamine, stearylamine, oleylamine, and benzylamine.

30 Examples of the secondary amine include diethylamine, diisopropylamine, dibutylamine, dipentylamine, dihexylamine, dicyclohexylamine, diocetylamine, dilaurylamine, distearylamine, dioleylamine, dibenzylamine, diethanolamine, 35 piperazine, diisopropanolamine, stearylethanolamine, decylenethanolamine, hexylpropanolamine, benzylethanolamine, phenylethanolamine, and tolylpropanolamine.

35 Examples of the tertiary amine include tributylamine, tripentylamine, trihexylamine, tricyclohexylamine, trioctylamine, trilaurylamine, tristearylamine, trioleylamine, tribenzylamine, methyldicyclohexylamine, dioleylethanolamine, dilaurylpropanolamine, diocylethanolamine, dibutylethanolamine, diethylethanolamine, dimethylethanolamine, 40 dihexylpropanolamine, dibutylpropanolamine, oleyldiethanolamine, stearylidipropanolamine, lauryldiethanolamine, octyldipropanolamine, butyldiethanolamine, methyldiethanolamine, cyclohexyldiethanolamine, benzylidethanolamine, phenyldiethanolamine, tolyldipropanolamine, 45 xylidethanolamine, triethanolamine, tripropylamine, and triisopropanolamine.

50 These amine compounds form amine salts with a carboxylic acid serving as the component C. When the water-soluble metal-working oil agent contains an amine compound, the stability of the water-soluble metal-working oil agent is ensured, and water solubility thereof can be improved. From the viewpoints of emulsion stability, anti-corrosiveness, and rotting resistance, the amine compound used in the invention is preferably an alkanolamine and/or an alkylamine.

55 Notably, base value (hydrochloric acid method) is determined in accordance with JIS K2501.

## &lt;Water&gt;

The water-soluble metal-working oil agent (undiluted liquid composition) may contain a certain amount of water. From the viewpoint of water solubility, the amount of water with respect to the entire amount of the water-soluble metal-working oil agent is preferably 0 to 50 mass %, more preferably 3 to 45 mass %, still more preferably 6 to 40 mass %.

## &lt;Other Additional Components&gt;

The water-soluble metal-working oil agent may further contain other components, so long as the effects of the present invention are not impaired. Examples of such additional components include a surfactant, a lubricity improver, a metal deactivator, a defoaming agent, an antiseptic, and an anti-oxidant.

Examples of the surfactant include an anionic surfactant, a cationic surfactant, a nonionic surfactant, and an amphoteric surfactant. Examples of the anionic surfactant include alkylbenzenesulfonate salts and  $\alpha$ -olefinsulfonate salts. Examples of the cationic surfactant include quaternary ammonium salts such as alkyltrimethylammonium salts, dialkyldimethylammonium salts, and alkylidimethylbenzylammonium salts. Examples of the nonionic surfactant include ethers such as polyoxyethylene alkyl ether and polyoxyethylene alkylphenyl ether; esters such as sorbitan fatty acid ester, polyoxyethylene sorbitan fatty acid ester, and polyoxyethylene fatty acid ester; and amides such as fatty acid alkanolamide. Examples of the amphoteric surfactant include betaines such as alkylbetain.

Examples of the lubricity improver include organic acids. Specific examples of such organic acids include caprylic acid, pelargonic acid, isononanoic acid, capric acid, lauric acid, stearic acid, oleic acid, benzoic acid, p-tert-butylbenzoic acid, adipic acid, suberic acid, sebacic acid, azelaic acid, and dodecanoic acid.

Examples of the metal deactivator include benzotriazole, imidazoline, primidine derivatives, and thiadiazole.

Examples of the anti-oxidant include amine-type antioxidants such as alkylated diphenylamine, phenyl- $\alpha$ -naphthylamine, and alkylated phenyl- $\alpha$ -naphthylamine; phenol-type anti-oxidants such as 2,6-di-t-butylphenol, 4,4'-methylenebis(2,6-di-t-butylphenol), isoocetyl-3-(3,5-di-t-butyl-4-hydroxyphenyl)propionate, and n-octadecyl-3-(3,5-di-t-butyl-4-hydroxyphenyl)propionate; sulfur-type anti-oxidants such as dilauryl-3,3'-thiodipropionate; phosphorus-type anti-oxidants such as phosphite; and molybdenum-type antioxidants.

Examples of the antiseptic include a triazine-based antiseptic and an alkylbenzimidazole-based antiseptic.

Examples of the defoaming agent include methylsilicone oil, fluorosilicone oil, and polyacrylate.

## [Metal-Working Liquid]

The metal-working liquid of the present invention is produced by diluting the water-soluble metal-working oil agent (undiluted liquid composition) with water. No particular limitation is imposed on the water, and any of distilled water, ion-exchange water, and tap water may be employed. The water-soluble metal-working oil agent concentration of the diluted product is preferably 3 vol. % to 20 vol. %, more preferably 5 vol. % or higher, still more preferably 10 vol. % or higher. When the diluted product has an oil agent concentration lower than 3 vol. %, sufficient workability may fail to be attained, whereas when the concentration is in

excess of 20 vol. %, stability of the diluted product may be impaired.

## [Metal-Working Method]

The metal-working method of the present invention includes working a metal workpiece by use of the water-soluble metal-working oil agent (undiluted liquid composition) or the metal-working liquid formed of the water-soluble metal-working oil agent diluted by water. Examples of the metal working process to which the method of the invention may be applied include various metal machining processes such as cutting, grinding, punching, polishing, deep drawing, drawing, and rolling. The metal-working agent of the present invention, providing excellent lubricity, is suitable for machining a so-called hard-to-work material.

The metal forming the workpiece includes a pure metal composed of a single metal element, a mixture of a plurality of metal elements, and a mixture of a metal element and a non-metallic element. The hard-to-work material is at least one species selected from the group consisting of titanium, titanium alloy, nickel alloy, niobium alloy, tantalum alloy, molybdenum alloy, tungsten alloy, stainless steel, and high-manganese steel.

According to the metal-working method of the present invention, a metal working agent which does not contain a compound containing chlorine, sulfur, or phosphorus can be suitably used in intermittent cutting, such as end milling, of a hard-to-work material.

## EXAMPLES

The present invention will next be described in more detail by way of examples, which should not be construed as limiting the invention thereto. Characteristics of samples of the water-soluble metal-working oil agent according to the Examples and Comparative Examples were evaluated through the following methods.

## [Evaluation Methods]

## &lt;Evaluation of Stability of Undiluted Liquid&gt;

The stability of undiluted liquid samples of the water-soluble metal-working oil agent (undiluted liquid composition) was evaluated. Specifically, each of the water-soluble metal-working oil agents obtained in the Examples and Comparative Examples was allowed to stand at 25° C. for 24 hours, and phase separation was checked. A sample in which no separation was observed is rated as "O," and a sample in which separation was observed is rated as "X."

## &lt;Cutting Performance Evaluation&gt;

Cutting performance was evaluated by tool life. Firstly, a workpiece was subjected to end milling by means of an upright machining center under the following conditions. Tool life is defined as the shorter of two periods: a period of time from start of cutting to the point in time when the abrasion of the flank exceeded 0.2 mm, and a period of time from start of cutting to the point in time when the tool was damaged. Each water-soluble metal-working oil agent (undiluted liquid composition) was diluted with water, to thereby prepare a 10 vol. % metal-working liquid, which was employed in cutting performance evaluation.

Facility: upright machining center NV 5000α1/A40, Moroseiki

Work piece: Ti-6Al-4V,  $\phi$ 150×30 mm, disk shape  
Insert: XOMX 090308 TR-ME06, F40M (type S30), product of SECO TOOLS

Cutter: Helical Micro Turbo R217.69-2020.3-016-09.2, product of SECO TOOLS

Holder: HSK63A milling chuck CT20A, product of NT Tool  
Cutting speed: 80 m/min, 55 m/min

## 9

Cut-out: ap (tool axial direction): 2 mm, ae (tool radial direction): 16 mm

Feed: 0.1 mm/tooth

Oil feed: external feed, 3.7 L/min

Dilution: 10 vol. % (dilution by water)

[Component A]

Characteristics of the mineral oils employed as the component A are as follows.

<Mineral Oil 1 (Component A1)>

Naphthene Base Mineral Oil

Characteristic temperature: 597° C., kinematic viscosity (40° C.): 434 mm<sup>2</sup>/s, kinematic viscosity (100° C.): 21 mm<sup>2</sup>/s, viscosity index: 35, density (15° C.): 0.9270, and flash point: 246° C.

The characteristic temperature of mineral oil was determined in accordance with JIS K2242, heat-treating oil quench test (method A). The kinematic viscosity of mineral oil was determined in accordance with JIS K2283. The density of mineral oil was determined in accordance with JIS K2249. The flash point of mineral oil was determined in accordance with JIS K2265-4 (COC method).

<Mineral Oil 2 (Component A2)>

Naphthene Base Mineral Oil

Characteristic temperature: 534° C., kinematic viscosity (40° C.): 101 mm<sup>2</sup>/s, kinematic viscosity (100° C.): 9 mm<sup>2</sup>/s, viscosity index: 43, density (15° C.): 0.9011, and flash point: 212° C.

<Mineral Oil 3 (Component A3)>

Characteristic temperature: 496° C., kinematic viscosity (40° C.): 47 mm<sup>2</sup>/s, kinematic viscosity (100° C.): 6 mm<sup>2</sup>/s, viscosity index: 26, density (15° C.): 0.9205, and flash point: 174° C.

<Ester Compound (Component A4)>

Pentaerythritol Tetraester

Characteristic temperature: 558° C., kinematic viscosity (40° C.): 34 mm<sup>2</sup>/s, kinematic viscosity (100° C.): 6 mm<sup>2</sup>/s, viscosity index: 126, density (15° C.): 0.9610, and flash point: 280° C.

[Component B]

<Condensed Fatty Acid 1 (Component B1)>

Ricinoleic acid was subjected to heat dehydration-condensation at 200° C. under a flow of nitrogen, to thereby yield condensed fatty acid 1. The condensed fatty acid 1 had a characteristic temperature of 712° C., an acid value: 34 mgKOH/g, a hydroxyl value of 28 mgKOH/g, and a saponification value of 198 mgKOH/g.

The acid value was determined in accordance with JIS K2501. The hydroxyl value was determined in accordance with JIS K0070. The saponification value was determined in accordance with JIS K2503.

## 10

<Condensed Fatty Acid 2 (Component B2)>

Ricinoleic acid was subjected to heat dehydration-condensation at 200° C. under a flow of nitrogen, to thereby yield condensed fatty acid 2. The condensed fatty acid 2 had a characteristic temperature: 680° C., an acid value: 53 mgKOH/g, a hydroxyl value: 42 mgKOH/g, and a saponification value: 196 mgKOH/g.

<Condensed Fatty Acid 3 (Component B3)>

Ricinoleic acid was subjected to heat dehydration-condensation at 200° C. under a flow of nitrogen, and the product was further subjected to heat dehydration-condensation with oleic acid, to thereby yield condensed fatty acid 3. The condensed fatty acid 3 had a characteristic temperature of 666° C., an acid value of 55 mgKOH/g, a hydroxyl value of 9 mgKOH/g, and a saponification value of 201 mgKOH/g.

<Condensed Fatty Acid 4 (Component B4)>

Ricinoleic acid was subjected to heat dehydration-condensation at 200° C. under a flow of nitrogen, and the product was further subjected to heat dehydration-condensation with oleic acid, to thereby yield condensed fatty acid 4. The condensed fatty acid 4 had a characteristic temperature of 628° C., an acid value of 85 mgKOH/g, a hydroxyl value of 15 mgKOH/g, and a saponification value of 195 mgKOH/g.

[Component C]

<Carboxylic Acid 1 Component C1>

Oleic acid, acid value: 198 mgKOH/g

<Carboxylic Acid 2 Component C2>

Neodecanoic acid, acid value: 321 mgKOH/g

<Carboxylic Acid 3 Component C3>

Sebacic acid, acid value: 554 mgKOH/g

[Component D]

<Amine 1 (Component D1)>

Monoisopropanolamine, base value: 747 mgKOH/g

<Amine 2 (Component D2)>

Methyldicyclohexylamine, base value: 284 mgKOH/g

The base value (hydrochloric acid method) was determined in accordance with JIS K2501.

## EXAMPLES AND COMPARATIVE EXAMPLES

According to the formulations shown in Table 1, components were mixed to prepare water-soluble metal-working oil agents. The water-soluble metal-working oil agents produced in Examples 1 to 7, and those produced in Comparative Examples 1 to 6 were evaluated through the aforementioned methods. Table 1 shows the results.

TABLE 1

| Components        | Water-soluble<br>by<br>mass) | A<br>metal-<br>working<br>oil<br>agent | B   | C   | Kinematic<br>viscosity<br>40° C. | Charact.<br>temp.<br>(° C.) | (mm <sup>2</sup> /s) | Acid<br>value<br>(mgKOH/g) | OH<br>value<br>(mgKOH/g) | Base<br>value<br>(mgKOH/<br>g) | Examples |      |      |      |   |
|-------------------|------------------------------|----------------------------------------|-----|-----|----------------------------------|-----------------------------|----------------------|----------------------------|--------------------------|--------------------------------|----------|------|------|------|---|
|                   |                              |                                        |     |     |                                  |                             |                      |                            |                          |                                | 1        | 2    | 3    | 4    | 5 |
| Mineral oil 1     | A1                           | 597                                    | 434 | —   | —                                | —                           | —                    | —                          | —                        | 20.0                           | 20.0     | 54.0 | 20.0 | 20.0 |   |
| Mineral oil 2     | A2                           | 534                                    | 101 | —   | —                                | —                           | —                    | —                          | —                        | —                              | —        | —    | —    | —    |   |
| Mineral oil 3     | A3                           | 496                                    | 47  | —   | —                                | —                           | —                    | —                          | —                        | —                              | —        | —    | —    | —    |   |
| Ester 1           | A4                           | 558                                    | 34  | —   | —                                | —                           | —                    | —                          | —                        | —                              | —        | —    | —    | —    |   |
| C. fatty acid 1   | B1                           | 712                                    | —   | 34  | 28                               | —                           | 15.0                 | 15.0                       | 10.0                     | 10.0                           | —        | —    | —    | —    |   |
| C. fatty acid 2   | B2                           | 680                                    | —   | 53  | 42                               | —                           | —                    | —                          | —                        | —                              | —        | —    | —    | 17.0 |   |
| C. fatty acid 3   | B3                           | 666                                    | —   | 55  | 9                                | —                           | —                    | —                          | —                        | —                              | —        | —    | —    | —    |   |
| C. fatty acid 4   | B4                           | 628                                    | —   | 85  | 15                               | —                           | —                    | —                          | —                        | —                              | —        | —    | —    | —    |   |
| Carboxylic acid 1 | C1                           | —                                      | —   | 198 | —                                | —                           | 3.0                  | 3.0                        | 7.0                      | 3.0                            | 14.0     | —    | —    | —    |   |
| Carboxylic acid 2 | C2                           | —                                      | —   | 321 | —                                | —                           | 6.5                  | 6.5                        | —                        | 6.5                            | 6.5      | —    | —    | —    |   |
| Carboxylic acid 3 | C3                           | —                                      | —   | 554 | —                                | —                           | 3.5                  | 3.5                        | 3.0                      | 3.5                            | 3.5      | —    | —    | —    |   |

TABLE 1-continued

|                                        |                                     |                 |            |   |   |   |     |      |       |      |      |      |
|----------------------------------------|-------------------------------------|-----------------|------------|---|---|---|-----|------|-------|------|------|------|
| D                                      | Amine 1                             | D1              | —          | — | — | — | 747 | 11.0 | 11.0  | 5.0  | 11.0 | 11.0 |
|                                        | Amine 2                             | D2              | —          | — | — | — | 284 | 6.5  | 6.5   | 9.0  | 6.5  | 6.5  |
|                                        | Benzotriazole                       |                 |            |   |   |   |     | 1.0  | 1.0   | 1.0  | 1.0  | 1.0  |
|                                        | Polyoxyethylene monoalkyl ether     |                 |            |   |   |   |     | 2.0  | 2.0   | —    | 2.0  | 2.0  |
|                                        | Polyoxyethylene sorbitan monooleate |                 |            |   |   |   |     | —    | —     | 3.0  | —    | —    |
|                                        | Water                               |                 |            |   |   |   |     | 31.5 | 31.5  | 8.0  | 36.5 | 18.5 |
| Acid value (component B + component C) |                                     |                 |            |   |   |   |     | 51   | 51    | 34   | 50   | 77   |
| Base value (component D)               |                                     |                 |            |   |   |   |     | 101  | 101   | 63   | 101  | 101  |
| Test conditions                        | Cutting speed                       | 55 (m/min)      | 80 (m/min) |   |   |   |     | —    | ○     | —    | —    | —    |
| Evaluation results                     | Undiluted liquid stability          | Tool life (min) |            |   |   |   |     | ○    | —     | ○    | ○    | ○    |
|                                        |                                     |                 |            |   |   |   |     | ○    | ○     | ○    | ○    | ○    |
|                                        |                                     |                 |            |   |   |   |     | 20.3 | >50.0 | 22.4 | 18.3 | 16.2 |

|                               |                                                     |    | Charact.<br>temp.                      | Kinematic<br>viscosity     |            | Acid<br>value        | OH<br>value | Base<br>value | Examples  |      | Comp. Exs. |      |      |
|-------------------------------|-----------------------------------------------------|----|----------------------------------------|----------------------------|------------|----------------------|-------------|---------------|-----------|------|------------|------|------|
|                               |                                                     |    |                                        | 40° C.                     | (° C.)     | (mm <sup>2</sup> /s) | (mgKOH/g)   | (mgKOH/g)     | (mgKOH/g) | 6    | 7          | 1    | 2    |
| Components<br>(parts by mass) | Water-<br>soluble<br>metal-<br>working<br>oil agent | A  | Mineral oil 1                          | A1                         | 597        | 434                  | —           | —             | —         | 20.0 | 20.0       | —    | —    |
|                               |                                                     |    | Mineral oil 2                          | A2                         | 534        | 101                  | —           | —             | —         | —    | —          | 20.0 | —    |
|                               |                                                     | B  | Mineral oil 3                          | A3                         | 496        | 47                   | —           | —             | —         | —    | —          | —    | 20.0 |
|                               |                                                     |    | Ester 1                                | A4                         | 558        | 34                   | —           | —             | —         | —    | —          | —    | —    |
|                               |                                                     |    | C. fatty acid 1                        | B1                         | 712        | —                    | 34          | 28            | —         | —    | —          | 15.0 | 15.0 |
|                               | C                                                   | C. | fatty acid 2                           | B2                         | 680        | —                    | 53          | 42            | —         | 17.0 | —          | —    | —    |
|                               |                                                     |    | fatty acid 3                           | B3                         | 666        | —                    | 55          | 9             | —         | —    | 15.0       | —    | —    |
|                               |                                                     | C  | fatty acid 4                           | B4                         | 628        | —                    | 85          | 15            | —         | —    | —          | —    | —    |
|                               |                                                     |    | Carboxylic acid 1                      | C1                         | —          | —                    | 198         | —             | —         | 14.0 | 3.0        | 3.0  | 3.0  |
|                               |                                                     |    | Carboxylic acid 2                      | C2                         | —          | —                    | 321         | —             | —         | 6.5  | 6.5        | 6.5  | 6.5  |
|                               | D                                                   | D  | Carboxylic acid 3                      | C3                         | —          | —                    | 554         | —             | —         | 3.5  | 3.5        | 3.5  | 3.5  |
|                               |                                                     |    | Amine 1                                | D1                         | —          | —                    | —           | —             | 747       | 11.0 | 11.0       | 11.0 | 11.0 |
|                               |                                                     | D  | Amine 2                                | D2                         | —          | —                    | —           | —             | 284       | 6.5  | 6.5        | 6.5  | 6.5  |
|                               |                                                     |    | Benzotriazole                          | —                          | —          | —                    | —           | —             | —         | 1.0  | 1.0        | 1.0  | 1.0  |
|                               | E                                                   | E  | Polyoxyethylene monoalkyl ether        | —                          | —          | —                    | —           | —             | —         | 2.0  | 2.0        | 2.0  | 2.0  |
|                               |                                                     |    | Polyoxyethylene sorbitan monooleate    | —                          | —          | —                    | —           | —             | —         | —    | —          | —    | —    |
|                               |                                                     | E  | Water                                  | —                          | —          | —                    | —           | —             | —         | 18.5 | 31.5       | 31.5 | 31.5 |
|                               |                                                     |    | Acid value (component B + component C) | —                          | —          | —                    | —           | —             | —         | 77   | 54         | 51   | 51   |
|                               | F                                                   | F  | Base value (component D)               | —                          | —          | —                    | —           | —             | —         | 101  | 101        | 101  | 101  |
|                               |                                                     |    | Test conditions                        | Cutting speed              | 55 (m/min) | 80 (m/min)           | —           | —             | —         | ○    | —          | —    | —    |
|                               |                                                     | F  | Evaluation results                     | Undiluted liquid stability |            | —                    | —           | —             | ○         | ○    | ○          | ○    | ○    |
|                               |                                                     |    | Tool life (min)                        | —                          | —          | —                    | —           | —             | >50.0     | 18.3 | 6.1        | 6.1  | 6.1  |

|                                                       |                                                        |                                     |                   | Charact.<br>temp. | Kinematic<br>viscosity |                      | Acid<br>value | OH<br>value | Base<br>value | Comp. Exs. |      |      |      |
|-------------------------------------------------------|--------------------------------------------------------|-------------------------------------|-------------------|-------------------|------------------------|----------------------|---------------|-------------|---------------|------------|------|------|------|
|                                                       |                                                        |                                     |                   |                   | (° C.)                 | (mm <sup>2</sup> /s) |               |             |               | 3          | 4    | 5    | 6    |
| Components<br>(parts<br>by<br>mass)                   | Water-<br>soluble<br>metal-<br>working<br>oil<br>agent | A                                   | Mineral oil 1     | A1                | 597                    | 434                  | —             | —           | —             | —          | —    | —    | 20.0 |
|                                                       |                                                        |                                     | Mineral oil 2     | A2                | 534                    | 101                  | —             | —           | —             | —          | —    | —    | —    |
|                                                       |                                                        | B                                   | Mineral oil 3     | A3                | 496                    | 47                   | —             | —           | —             | —          | —    | —    | —    |
|                                                       |                                                        |                                     | Ester 1           | A4                | 558                    | 34                   | —             | —           | —             | 20.0       | 20.0 | 20.0 | —    |
|                                                       |                                                        |                                     | C. fatty acid 1   | B1                | 712                    | —                    | 34            | 28          | —             | 15.0       | —    | —    | —    |
|                                                       | C                                                      | C                                   | C. fatty acid 2   | B2                | 680                    | —                    | 53            | 42          | —             | —          | —    | —    | —    |
|                                                       |                                                        |                                     | C. fatty acid 3   | B3                | 666                    | —                    | 55            | 9           | —             | —          | —    | —    | —    |
|                                                       |                                                        | C                                   | C. fatty acid 4   | B4                | 628                    | —                    | 85            | 15          | —             | —          | 15.0 | 15.0 | 17.0 |
|                                                       |                                                        |                                     | Carboxylic acid 1 | C1                | —                      | —                    | 198           | —           | —             | 3.0        | 3.0  | 3.0  | 6.0  |
|                                                       |                                                        |                                     | Carboxylic acid 2 | C2                | —                      | —                    | 321           | —           | —             | 6.5        | 6.5  | 6.5  | 6.5  |
|                                                       | D                                                      | D                                   | Carboxylic acid 3 | C3                | —                      | —                    | 554           | —           | —             | 3.5        | 3.5  | 3.5  | 3.5  |
|                                                       |                                                        |                                     | Amine 1           | D1                | —                      | —                    | —             | —           | 747           | 11.0       | 11.0 | 11.0 | 11.0 |
|                                                       |                                                        | D                                   | Amine 2           | D2                | —                      | —                    | —             | —           | 284           | 6.5        | 6.5  | 6.5  | 6.5  |
|                                                       |                                                        |                                     | Benzotriazole     | —                 | —                      | —                    | —             | —           | —             | 1.0        | 1.0  | 1.0  | 1.0  |
| Acid value (component B +<br>Base value (component D) | Test<br>conditions                                     | Polyoxyethylene monoalkyl ether     |                   |                   |                        | —                    | —             | —           | —             | 2.0        | 2.0  | 2.0  | 2.0  |
|                                                       |                                                        | Polyoxyethylene sorbitan monooleate |                   |                   |                        | —                    | —             | —           | —             | —          | —    | —    | —    |
|                                                       |                                                        | Water                               |                   |                   |                        | —                    | —             | —           | —             | 31.5       | 31.5 | 31.5 | 26.5 |
|                                                       |                                                        | Cutting speed                       |                   |                   |                        | 55 (m/min)           | —             | —           | —             | 51         | 67   | 67   | 67   |
|                                                       |                                                        | 80 (m/min)                          |                   |                   |                        | —                    | —             | —           | —             | 101        | 101  | 101  | 101  |
| Evaluation<br>results                                 | Undiluted liquid stability                             |                                     |                   |                   | —                      | —                    | —             | —           | —             | —          | —    | —    | —    |
|                                                       | Tool life (min)                                        |                                     |                   |                   | —                      | —                    | —             | —           | —             | —          | —    | —    | —    |
|                                                       | 10.2                                                   |                                     |                   |                   | 6.1                    | 47                   | —             | —           | —             | —          | —    | —    | 8.1  |

C. fatty acid: condensed fatty acid

## [Evaluation Results]

As is clear from Table 1, the water-soluble metal-working oil agents falling within the scope of the present invention provided a longer tool life in machining a workpiece made

of Ti-6AL-4V, which is a hard-to-work material, as compared with the water-soluble metal-working oil agents of the Comparative Examples. Water-soluble metal-working oil agents containing a component having a characteristic tem-

## 13

perature below a target level, and water-soluble metal-working oil agents containing a component having a characteristic temperature satisfying a target level in an amount below the target amount satisfied the target stability in the undiluted state, but did not satisfy the target for tool life. Water-soluble metal-working oil agents containing the component C or the component D in an amount falling outside the target range did not ensure the target stability in the undiluted state.

The water-soluble metal-working oil agent of Comparative Example 5 provided a tool life of about 47 min, when the cutting speed was 55 m/min, but when the cutting speed was elevated to 80 m/min (about 1.5 times) (i.e., Comparative Example 4), the tool life was considerably impaired.

In contrast, the water-soluble metal-working oil agents of Examples 2 and 6 exhibited equivalent or more excellent performance in the case of low-speed cutting, as compared with the water-soluble metal-working oil agent of Comparative Example 5, and attained a target tool life even at a cutting speed of 80 m/min. Thus, through selection of the mineral oil on the basis of characteristic temperature defined in JIS K2242, and selection of a specific condensed fatty acid, a remarkably prolonged tool life was realized in metal working; i.e., intermittent cutting, of a hard-to-work material at a cutting speed faster than a conventionally employed cutting speed.

The invention claimed is:

1. A water-soluble metal-working oil agent, comprising:
  - (A) a naphthalene base mineral oil having
    - a characteristic temperature, as measured in accordance with JIS K2242, of 570° C. or higher,
    - a kinematic viscosity, as determined at 40° C. in accordance with JIS K2283, of 300 mm<sup>2</sup>/s or higher, and
    - a flash point of 220° C. or higher;
  - (B) at least one condensed fatty acid selected from the group consisting of
    - a condensed fatty acid (1) produced through dehydration condensation of a hydroxycarboxylic acid, and
    - a condensed fatty acid (2) produced through dehydration condensation of an alcoholic hydroxyl group of the condensed fatty acid (1) with a monovalent carboxylic acid, which has a characteristic temperature, as measured in accordance with JIS K2242, of 650° C. or higher; and
  - a surfactant,
- wherein the condensed fatty acid (B) is present in an amount of 7.5 mass % or more to 17 mass % with respect to an entire amount of the oil agent.
2. The oil agent according to claim 1, wherein the mineral oil (A) has a kinematic viscosity of 400 mm<sup>2</sup>/s or higher and 500 mm<sup>2</sup>/s or lower, and
  - wherein the mineral oil has a flash point of 230° C. or higher.
  3. The oil agent according to claim 1, wherein the mineral oil (A) is present in an amount of 10 mass % or more with respect to an entire amount of the oil agent.

## 14

4. The oil agent according to claim 1, wherein the condensed fatty acid (B) is the condensed fatty acid (1) produced through dehydration condensation of ricinoleic acid.
5. The oil agent according to claim 1, wherein the condensed fatty acid (B) has an acid value of 60 mgKOH/g or less and a hydroxyl value of 50 mgKOH/g or less.
6. The oil agent according to claim 1, further comprising: (C) a carboxylic acid.
7. The oil agent according to claim 6, wherein the carboxylic acid (C) is present in an amount of 2 mass % or more with respect to an entire amount of the oil agent.
8. The oil agent according to claim 6, further comprising: (D) an amine compound or an alkali metal compound.
9. The oil agent according to claim 8, wherein the amine compound or an alkali metal compound (D) is present in such a neutralization equivalent that at least the condensed fatty acid (B) and the carboxylic acid (C) are neutralized to cancel out a sum of the acid values thereof.
10. The oil agent according to claim 8, comprising the amine compound (D), which is at least one of an alkanolamine and an alkylamine.
11. The oil agent according to claim 1, further comprising: water.
12. A metal-working liquid comprising: the oil agent according to claim 1, wherein the oil agent is diluted by water.
13. A metal-working method, comprising: working a metal workpiece using the oil agent according to claim 1.
14. A metal-working method, comprising: working a metal workpiece using the metal-working liquid according to claim 12.
15. The metal-working method according to claim 13, wherein the metal workpiece is at least one selected from the group consisting of titanium, titanium alloy, nickel alloy, niobium alloy, tantalum alloy, molybdenum alloy, tungsten alloy, stainless steel, and high-manganese steel.
16. The metal-working method according to claim 13, which is intermittent cutting.
17. The oil agent according to claim 8, comprising, based on the entire amount of the oil agent:
  - 15 mass % of the mineral oil (A);
  - from 10 mass % or more to 17 mass % of the condensed fatty acid (B), which is the condensed fatty acid (1) produced through dehydration condensation of ricinoleic acid;
  - 8 mass % or more of the carboxylic acid (C);
  - an amine compound (D), which is at least one of an alkanolamine and an alkylamine; and
  - 6 to 40% of water.
18. The oil agent according to claim 1, wherein the surfactant is a nonionic surfactant.
19. The oil agent according to claim 18, wherein the nonionic surfactant is at least one selected from the group consisting of a polyoxyethylene alkyl ether, a polyoxyethylene alkylphenyl ether, a sorbitan fatty acid ester, and a polyoxyethylene sorbitan fatty acid ester.

\* \* \* \* \*